

No. 773,368.

PATENTED OCT. 25, 1904.

G. BOWER & F. W. GAUNTLETT.

SUBSTITUTE FOR LITHOGRAPHIC STONES AND METHOD OF MAKING SAME.

APPLICATION FILED FEB. 23, 1904.

NO MODEL.



Witnesses,

James L. Morris, Jr.  
C. S. Kessler

Inventors

George Bower  
Frederick W. Gauntlett  
James L. Morris  
Atty.

## UNITED STATES PATENT OFFICE.

GEORGE BOWER, OF ST. NEOTS, AND FREDERICK WILLIAM GAUNTLETT,  
OF LONDON, ENGLAND.

## SUBSTITUTE FOR LITHOGRAPHIC STONES AND METHOD OF MAKING SAME.

SPECIFICATION forming part of Letters Patent No. 773,368, dated October 25, 1904.

Application filed February 23, 1904. Serial No. 194,874. (No model.)

*To all whom it may concern:*

Be it known that we, GEORGE BOWER, residing at The Shrubbery, St. Neots, Hunts, and FREDERICK WILLIAM GAUNTLETT, residing at 2 Tower Royal, Cannon street, London, England, subjects of the King of Great Britain, have invented certain new and useful Improvements in Substitutes for Lithographic Stones and Methods of Making the Same, of which the following is a specification.

The object of this invention is to provide substitutes for the stones which are commonly used for lithographic purposes and which have surfaces equal to or superior to those of the stones and at the same time have the flexibility of the sheets of metal which have also been used for the same purpose and which are especially suitable both for flat-bed and rotary machines. In order to accomplish this, we take metallic sheets and either convert the surfaces of such sheets into an oxid of the same metal or else we form an oxid of another metal upon the said metallic sheets, or we may form both oxids at the same time, if desired, or, again, we may convert the surface of the metallic sheet into an oxid and over this form oxids of two or more metals. In any case the oxid or oxids are made to form tenacious coatings to the metallic sheets, and such oxids by their nature take the lithographic ink readily and are sufficiently absorbent and flexible as to stand bending round the smallest cylinders which are used or likely to be used in printing-machines.

By one method we take sheets of iron or steel and convert the surfaces thereof into an oxid or combination of oxids of iron by the action of heat and steam which may be advantageously superheated or by the action of the heat and air or products of combustion, or in any of the ways in which iron or steel may be oxidized so as to form a firm adherent coating of oxid to the metal itself. Preferably we so oxidize the iron or steel that it may have a light French gray color and be more or less of the nature of the magnetic oxid of iron, which is also a preservative against the formation of the red oxid or common rust, and therefore of especial value. This coating of oxid

is flexible to a considerable degree, and so does not separate from the iron or steel sheets when they are bent, and, moreover, for lithographic and printing purposes the surfaces presented by such oxids are equal or superior to those of the best stones. Or we may form an oxid or oxids of one or more other metals upon the metallic sheets by chemical means with the application of heat. As an example, iron or steel may be dipped into a cupric salt, such as the sulfate or nitrate of copper, when if the sheets of iron or steel be clean an even layer of metallic copper is formed upon them, which by the application of heat in an oxidizing atmosphere may be converted into an oxid of copper of the desired color, texture, and tenacity, or the copper or other metals may be deposited by the aid of electricity upon such other metallic sheets as may be desirable and likewise converted into the porous and tenacious oxids which are desired. Or, yet again, the second metal, or it may be combination of metals, may be deposited upon the primary metallic sheets by the simple method of dipping, as is done in the manufacture of galvanized iron or steel or of tin plates.

In the case where iron or steel sheets are coated with zinc or zinc and tin combined and then the whole oxidized by heat in an oxidizing atmosphere of any convenient nature the result is metallic iron or steel in the interior of the sheet, oxid of iron on each side of this and closely adhering thereto, and externally films of the oxids of zinc or tin, or both, and firmly adherent to the oxid of iron. The oxids of zinc and tin are white in color—a point of considerable importance and value; but almost any suitable color may be produced by the use of different oxids.

Russian sheet-iron is simply a case where iron or steel sheets are partly oxidized in the process of manufacture and in no way evades the true spirit of our invention, which generally consists in the employment of metallic sheets and in the conversion of the surface of such sheets to an oxid or combination of oxids, which provides the necessary porosity and surface texture for lithographic-printing purposes, or otherwise coating the metallic sheets

primarily used with some other convenient 5  
oxid or oxids of the required porosity and  
texture, it being understood that the original  
sheets may also have their surfaces oxidized  
at the same time, if desired. In this manner  
we combine the advantages of the stones and  
the metallic sheets which have hitherto been  
employed and at the same time we eliminate  
the disadvantages which are common to either  
10 class of material by itself, for the oxid or  
combination of oxids, however produced, sup-  
plies the necessary surface and the metallic  
portion of the prepared sheet the required  
flexibility, and in order to show how our in-  
15 vention may be carried into effect we annex  
a sheet of drawings herewith, illustrating one  
method of producing the magnetic oxid and  
which has been in successful operation.

In the drawings, *a b* is a retort or muffle  
20 surrounded by brickwork *c c*. A gas-pipe *d*  
supplies a series of burners *e*, which play upon  
the bottom of the retort *a b*. The products  
of combustion escape through openings at *f*.  
A lid *g* is provided for the retort, and this is  
25 perforated with small holes.

*h* is a steam-pipe from a boiler, while *k* is a  
smaller pipe fitted with a funnel *l*, into which oil  
is allowed to drop, so that the oil ultimately  
mixes with the steam entering at *h*. The mix-  
30 ture then flows through the downright pipe *m*,  
which is heated, so that the oil becomes vapor-  
ized, and the steam and oil-vapor then pass  
along *n* to the longitudinal pipe *o*, which runs  
35 the whole length of the retort and is perforated  
with small holes at its lower portion, so that  
the oil-vapor and the steam are compelled to  
strike upon the heated bottom of the retort *a b*.  
The object of this is to insure that any free  
40 oxygen which may be with the steam shall be  
compelled to combine with the hydrocarbon  
vapor. After such combination the mixture  
passes through a mass of iron turnings or  
borings, as shown at *p*, and which are at a  
45 fairly high temperature. The steam now de-  
prived of any free oxygen, which it almost  
always has as ordinarily produced, passes  
upward through the sheets *q* of iron or steel,  
which are suspended in the retort or muffle  
50 *a b*, and by the decomposition of the steam  
the surfaces of the sheets are converted into  
magnetic oxid. The final exit of the differ-  
ent gases or vapors is through the holes in  
the lid *g* of the retort *a b*.

The object of the oil is to prevent any pos-  
55 sibility of the red oxid being formed upon

the sheets *q* instead of the magnetic oxid.  
A hydrocarbon vapor or combustible gas may  
be used instead of oil to eliminate the free  
oxygen; but oil is convenient and does its  
work well. The borings or turnings at *p* 60  
cause the steam to move upward evenly among  
the suspended sheets in the muffle, and this  
action is further aided by the perforations in  
the lid *g*.

The proper quantities of steam and oil 65  
which should pass over a given quantity of  
plates can only be determined by experiment;  
but when they are once properly proportioned  
the plates after two or three hours exposure  
at a scarcely visible red heat will be found to 70  
be coated with a firm adherent film of mag-  
netic oxid.

We have shown gas-burners for heating the  
retort; but of course solid fuel may be used,  
if convenient. 75

Sheets of iron or steel prepared as herein-  
before stated may be used for printing in  
precisely the same manner as lithographic  
stones are at present.

By the above methods we are enabled to 80  
produce plates having analogous surfaces to  
stones—viz., a surface which absorbs and re-  
tains grease and water. The want of this is  
the great drawback to zinc and aluminium  
and the cause from which most of the trouble 85  
incidental to their working arises.

What we claim, and desire to secure by Let-  
ters Patent, is—

1. A method of manufacturing a substitute 90  
for lithographic stones which consists in form-  
ing a metallic plate with a coating of oxid of  
metal to form a printing-surface by the sub-  
jecting of said plate in an oxidizing atmos-  
phere to the application of heat.

2. As a new article of manufacture, a sub- 95  
stitute for lithographic stones, consisting of  
a metallic plate having a printing-surface of  
oxid of iron.

3. As a new article of manufacture, a sub- 100  
stitute for lithographic stones, consisting of a  
metallic plate having a firmly adhering coating  
of oxid of iron forming a printing-surface.

In testimony whereof we have hereunto set  
our hands in presence of two subscribing wit-  
nesses.

GEORGE BOWER.

FREDERICK WILLIAM GAUNTLETT.

Witnesses:

W.M. O. BROWN,

FRED C. SMITH.